

# United States Patent Office

2,698,088

Patented Dec. 28, 1954

1

2,698,088

## SEPARATION OF MINERALS BY FROTH FLOTATION

Edmund James Pryor, Hendon, London, and Marston Greig Fleming and Stanislaw Aleksander Wrobel, London, England

No Drawing. Application April 26, 1952,  
Serial No. 284,648

Claims priority, application Great Britain March 11, 1952

### 10 Claims. (Cl. 209—166)

This invention relates to improvements in or relating to the separation of minerals by froth flotation.

For the efficient separation of ores by froth flotation, it is usually necessary or desirable to condition the surfaces of the small particles of the various minerals present in the "pulp," i. e. in the aqueous suspension of ore-particles produced by comminution. For this purpose "activating" and "depressing" chemicals are usually added, and these are usually followed by, or used contemporaneously with "collector" agents, the general effect being to develop a tendency in one type of particle to become aero-philic or hydrophobic and then to unite with passing air- or gas-bubbles which rise to the surface of the pulp and form a mineralised froth containing a high concentration of such particles, while at the same time the other particles in the pulp develop opposite characteristics or remain indifferent, so that most of them remain wetted in the pulp under the aerating or gasifying conditions which are extracting the aero-philic mineral.

For high efficiency of extraction, it is desirable that only small quantities of chemical be used, so as to aid their specific reaction with the particles; to maintain conditions in which these reagents are fully mobile and dispersed so that they can search the whole of the pulp; and to achieve a freely breaking froth when the mineralised bubbles rise, so that any hydrophilic particles which have become entrained in the froth can easily drop back into the pulp and thus do not contaminate the mineral being removed with the froth.

Commercial oleic acid, which is used industrially in large quantities as a collector agent in froth flotation processes, for example for separating fluorite ( $\text{CaF}_2$ ) from fluorspar ore, solidifies at about  $14^\circ \text{C}$ . It is generally necessary to heat the pulp far above this temperature in order to promote good dispersion of the collector agent during conditioning. There is the further difficulty that when the froth rises it may cool sufficiently for the oleic acid to freeze somewhat, thus producing a sullen froth which does not break or run freely, or a "flash-float" which forms and then can only be broken down with difficulty, thus locking up undesired mineral and reducing the purity of the desired product as well as increasing the difficulty of handling the frothed product. There is the further difficulty that when an envelope of frozen agent forms around any particle, that particle reacts to the formed surface and not to its inherent composition, so that particles which are by nature hydrophilic react under such circumstances as though they are hydrophobic, and thus are floated when it is desired that they remain sunk.

For these reasons it is desirable that collector agents should remain unfrozen at working temperatures. In the case of oleic acid this entails the introduction of heat into the flotation plant. This is costly, and can interfere with the reaction of the air or other gas with the pulp.

It is an object of this invention to provide a new oleic acid collector agent complex which is partly water-soluble and is wholly dispersed in the form of a stable emulsion on addition of water.

It is a further object to provide a new oleic acid collector agent complex which is a mobile dispersed agent at temperatures as low as  $5^\circ \text{C}$ . and confers high selectivity and excellent mobility upon the free running mineralised froth resulting from its use in flotation, even when quantities as small as 0.1% are used.

It is a still further object of this invention to provide a process for the production of the said new oleic acid collector agent complex.

Yet another object of this invention is to provide a

2

process for the separation of minerals by froth flotation employing the said new oleic acid collector agent complex.

Still another object of this invention is to provide a froth flotation process which enables calcium fluorite to be floated away from silica, shale, calcite and other minor contaminants in naturally occurring fluorspar ore in pulps produced during mill treatment using unheated water with the production of mineralised froths so clean that on drying they are found on assaying to contain more than 98%  $\text{CaF}_2$ .

The present invention provides a process for the production of a collector agent complex for use in the separation of minerals by froth flotation, which comprises making an aqueous dispersion of one part by weight of the free acids or the sodium salts of a mixture of petroleum sulphonated acids obtained by sulphonation of a high boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; mixing said aqueous dispersion (when the free acids are employed and preferably also when the sodium salts are employed) with an aqueous solution of one-third to 8 parts by weight of sodium silicate; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least  $50^\circ \text{C}$ ; and continuing agitation until the product is homogeneous on standing.

Preferably the substances specified above are employed in the following proportions by weight, calculated on 1 part by weight of the free acids or sodium salts of the mixture of petroleum sulphonated acids:

|                 |            |
|-----------------|------------|
| Sodium silicate | 0.5 to 5.0 |
| Water           | 15 to 50   |
| Oleic acid      | 10 to 50   |

The invention further provides a process for the separation of minerals by froth flotation wherein the collector agent produced by the above-described process is employed.

The properties of the collector agent complex are quite different from those of a mere mixture of its ingredients, and the flotation results obtainable with the complex are far superior to those obtainable with such a mere mixture. The conditions specified above have been found to be critical for the formation of the complex. Whilst we have no doubt that a complex is formed, as evidenced by the above-mentioned difference in properties, we have not been able to establish with certainty the mechanism involved. It appears that during the complex-formation the double bond of some of the oleic acid is saturated and that the complex formed assists in emulsifying the remainder of the oleic acid to give a highly active fluid collector agent.

The nature of the above-described sodium salts of petroleum sulphonated acids is discussed by Reuben Sparling in "Industrial and Engineering Chemistry," vol. 40 (1948), pages 890 et seq. Commercial petroleum sulphonates are available which contain these salts; they may be identified by their solubility in water, mineral hydrocarbon oils, oleic acid, benzene and chloroform, by their partial solubility in hydrochloric acid and by their formation of water-insoluble calcium and barium salts.

Among the proprietary organic compounds which contain varying and usually unspecified quantities of sulphonated hydrocarbon oils, we have tested the following during the development work which led to the establishment of the novel principles underlying the present invention. Our tests have shown that the following commercial sulphonates possess reactive powers in connection with the froth flotation of suitable ores:

Petromor Pale A, Petromor 276 and Petromor N, sold by Manchester Oil Refinery Ltd.  
R 824 and R825, sold by American Cyanamid Com-

## 3

pany, which behave substantially identically in the process of the invention.  
L M W, sold by Shell Chemicals Ltd.

The properties of these commercial products are tabulated below:

|   | Commercial product                          | Petromor Pale A   | Petromor 276      | Petromor N        | R 824, R 825      | L M W              |
|---|---------------------------------------------|-------------------|-------------------|-------------------|-------------------|--------------------|
| 1 | Solubility in H <sub>2</sub> O              | soluble           | soluble           | soluble           | soluble           | soluble.           |
| 2 | Solubility in hydrocarbon oil or oleic acid | do                | do                | do                | do                | Do.                |
| 3 | Solubility in benzene                       | do                | do                | do                | do                | Do.                |
| 4 | Solubility in chloroform                    | do                | do                | do                | do                | Do.                |
| 5 | Solubility in dilute hydrochloric acid      | partially soluble | partially soluble | partially soluble | partially soluble | partially soluble. |
| 6 | Solubility in Ca and Ba salts in water      | insoluble         | insoluble         | insoluble         | insoluble         | insoluble.         |
| 7 | Floatability Index with CaF <sub>2</sub>    | high              | high              | fair              | high              | very high.         |

The same commercial products, when converted into collector agent complexes with oleic acid by the process of the invention, exhibit the following properties:

|   | Commercial product                        | Petromor 276 | Petromor Pale A | Petromor N  | R 824 R 825 | L M W      |
|---|-------------------------------------------|--------------|-----------------|-------------|-------------|------------|
| 1 | Solubility or dispersibility in water     | good         | good            | good        | good        | good.      |
| 2 | Stability                                 | do           | fairly good     | fairly good | v. good     | v. good.   |
| 3 | Collecting power with CaF <sub>2</sub>    | v. good      | good            | fair        | do          | excellent. |
| 4 | Selectivity in CaF <sub>2</sub> flotation | do           | v. good         | good        | do          | Do.        |

In addition to the foregoing compounds, the following proprietary products were similarly tested. These contain sulphates or sulphonates other than the sodium petroleum sulphonates which are employed according to the present invention.

Vitanol and Petrosol, sold by Manchester Oil Refinery Ltd.

R 801, sold by American Cyanamid Company.

Teepol, sold by Shell Chemicals Ltd., which is stated to be a synthetic product based on sodium higher alkyl sulphates.

Sodium cetyl sulphate.

Limsopon 100 and Limsopon 574, sold by F. W. Berk & Co. Ltd., stated to be respectively a synthetic sulphate based on dodecyl benzene containing 35-40% of active ingredients.

The properties of these commercial products (which differ from the above-quoted properties of the commercial products suitable for use according to the invention) were proved by our tests to be as follows:

|   | Commercial product                          | Vitanol F. S. A.  | R 801             | Petrosol 33 | Teepol    | Limsopon 574 | Limsopon 100 |
|---|---------------------------------------------|-------------------|-------------------|-------------|-----------|--------------|--------------|
| 1 | Solubility in H <sub>2</sub> O              | partially soluble | soluble           | soluble     | soluble   | soluble      | soluble.     |
| 2 | Solubility in hydrocarbon oil or oleic acid | do                | partially soluble | insoluble   | insoluble | do           | Do.          |
| 3 | Solubility in benzene                       | soluble           | insoluble         | do          | do        | insoluble    | insoluble.   |
| 4 | Solubility in chloroform                    | partially soluble | partially soluble | do          | soluble   | soluble      | soluble.     |
| 5 | Solubility in dilute hydrochloric acid      | insoluble         | insoluble         | soluble     | soluble   | do           | Do.          |
| 6 | Solubility of Ba and Ca salts in water      | soluble           | soluble           | do          | insoluble | do           | Do.          |
| 7 | Floatability Index with CaF <sub>2</sub>    | low               | very low          | zero        | zero      | zero         | zero.        |

Attempts to convert these commercial products with oleic acid into collector agent complexes met with a complete lack of success, the mixtures having the following properties:

|   | Commercial product                     | Vitanol | R 801   | Petrosol 33 | Sodium Cetyl Sulphate | Teepol  | Limsopon 574 | Limsopon 100 |
|---|----------------------------------------|---------|---------|-------------|-----------------------|---------|--------------|--------------|
| 1 | Solubility or dispersibility in water  | none    | v. poor | none        | none                  | none    | none         | none.        |
| 2 | Stability                              | v. poor | do      | do          | v. poor               | do      | v. poor      | v. poor.     |
| 3 | Collecting power with CaF <sub>2</sub> | do      | do      | v. poor     | do                    | v. poor | do           | Do.          |

The collector agent complex produced by the process of the invention is partly water-soluble and is wholly dispersed in the form of a stable emulsion on addition of water.

4  
A number of additional modifying agents may be employed to facilitate manufacture or to enhance the frothing, collecting or selecting properties of the collector reagents (e. g. cresylic acid, pine oil, sodium silicate, quebracho). The quantity of each modifying agent

used, or of any combination of such agents should normally be made specific to the particular mineral which is to be treated, since interfacial (surface) reactions de-

pend upon a complex group of physical and chemical characteristics which vary even in naturally occurring ore-deposits of the same general type. Preferably the additional modifying agents are used in quantities of 5% or less of the weight of the long-chain fatty acid.

The following examples show how the process of the invention may be carried into effect:

## Example 1

P. F. 12.—2.0 gms. of R 825 were dissolved by heating in 10 gms. of water until the boiling point was reached. The mixture was immediately taken off the heat and added to 2.0 gms. of sodium silicate which was previously dissolved in 10 gms. of warm water. The resultant mixture was shaken for a few seconds to ensure homogeneity; 20 gms. of water were then added without further stirring, followed by immediate addition of 93.2 gms. of oleic acid which was previously heated above 60° C. in order to ensure its complete dissolution.

The total mixture (temp. 57° C.) was immediately shaken vigorously until chemical reaction was well set

in and the appearance and colour of the resultant complex-product changed from brown to creamy-white. 1.6 gms. of cresylic acid were then added and shaking continued for at least one hour or until the reaction was

substantially complete and the product appeared as a homogeneous thick fluid.

## Example 2

P. F. 6.—4.0 gms. of R 825 were dissolved by heating

in 20 gms. of water until the boiling point was reached. The mixture was immediately taken off the heat and added to 5.0 gms. of sodium silicate which had been previously dissolved in 30 gms. of warm water. The resultant mixture was shaken for a few seconds to ensure homogeneity; 50 gms. of water were then added without further stirring, followed by immediate addition of 40 gms. of oleic acid which was previously heated above 60° C. in order to ensure its complete dissolution.

The total mixture (temp. 55° C.) was immediately shaken vigorously until chemical reaction was well under way and the appearance and colour of the resultant complex-product changed from brown to creamy-white. The shaking was continued for at least one hour or until the reaction was complete and the product appeared as a homogeneous thick liquid.

#### Example 3

P. F. 8.—15.0 gms. of R 825 were dissolved by heating in 40 gms. of water until the boiling point was reached. The mixture was immediately taken off the heat and added to 5.0 gms. of sodium silicate which was previously dissolved in 30 gms. of warm water. The resultant mixture was shaken for a few seconds to ensure homogeneity; 50 gms. of water were added without further shaking, followed by immediate addition of 30 gms. of oleic acid which was previously heated above 60° C. in order to ensure its complete dissolution.

The total mixture (temp. 51° C.) was immediately shaken vigorously until chemical reaction was well under way and the appearance and colour of the resultant complex-product changed from brown to creamy-white. Shaking was continued for at least one hour or until the reaction was completed.

#### Example 4

P. F. 10.—2.0 gms. of R 825 were dissolved by heating in 10 gms. of water until the boiling point was reached. The mixture was immediately taken off the heat and added to 5.0 gms. of sodium silicate which was previously dissolved in 30 gms. of warm water. The resultant mixture was shaken for a few seconds to ensure homogeneity; 60 gms. of water were then added without further stirring, followed by immediate addition of 40 gms. of oleic acid which was previously heated to above 60° C. in order to ensure its complete dissolution.

The total mixture (temp. 53° C.) was immediately shaken vigorously until chemical reaction was completed (at least one hour) and the product appeared as a homogeneous liquid.

#### Example 5

P. F. 12 made with free sulphonic acid.—2.0 gms. (approximately) of free sulphonic acids liberated from R 825 were dissolved by heating in 10 gms. of water until the boiling point was reached. The mixture was immediately taken off the heat and added to 2.0 gms. of sodium silicate which was previously dissolved in 10 gms. of warm water. The resultant mixture was shaken for a few seconds to ensure homogeneity; 20 gms. of water were then added without further shaking, followed by immediate addition of 93.2 gms. of oleic acid which was previously heated above 60° C. in order to ensure its complete dissolution.

The total mixture (temp. 57° C.) was immediately shaken vigorously until chemical reaction was well set in and the appearance and colour of the resultant complex-product changed from brown to creamy-white. 1.6 gms. of cresylic acid were then added and shaking continued for at least one hour or until the reaction was substantially complete and the product appeared as a homogeneous thick liquid.

#### Example 6

P. F. 12 made without sodium silicate.—4.0 gms. of R 825 were dissolved by heating in 20 gms. of water until the boiling point was reached. The mixture was immediately taken off the heat. 20 gms. of water were added without stirring, followed by 93.2 gms. of oleic acid which was previously heated above 60° C. The total mixture (temp. 63° C.) was immediately shaken vigorously until chemical reaction was well set in and the appearance and colour of the resultant complex-product changed from brown to creamy-white. 1.6 gms. of cresylic acid were then added and shaking continued for at least one hour or until the reaction was substantially complete and the product appeared as a homogeneous thick liquid.

In the foregoing examples the degree of completion of the chemical reaction (depending upon the initial temperature at which mixing was carried out but which was above 50° C. and the total time of mixing the reactants) was tested by dropping a spot of the product into the water; if the reaction was complete, the drop of the reagent would rapidly dissolve with somewhat violent swirling; the failure or sluggishness of dissolution would indicate the need for further mixing in order to complete the desired reaction.

The conversion of oleic acid into a complex improves its fluidity dispersion in such a manner as to allow of improved commercial operation at lower temperatures. In laboratory tests it has been proved that a complex formed in this way from commercial oleic acid is a mobile dispersed agent at temperatures as low as 5° C. conferring high selectivity and excellent mobility upon the freely running mineralised froth resulting from its use in flotation even when quantities as small as 0.1% are used. It has been found possible to float calcium fluorite away from silica, shale, calcite and other minor contaminants in naturally occurring fluorspar ore in pulps produced during mill treatment using unheated water with the production of mineralised froths so clean that on drying they were found by assay to contain more than 98% CaF<sub>2</sub>, whereas when oleic acid was used in the conventional manner with standard conditioning agents such as quebracho, sodium silicate and alkali cyanide, similar ore could not be brought up to "acid grade" (+97.5% CaF<sub>2</sub>) without the use of temperatures exceeding 28° C. and repeated recleaning of the original froth.

In the full scale commercial tests referred to above assays were made at regular short intervals during four days of continuous operation and the following results were proved by assay:

|    | Mineral                 | Feed, percent | Concentrate, percent | Tailing, percent      |
|----|-------------------------|---------------|----------------------|-----------------------|
| 40 | CaF <sub>2</sub>        | 79.3          | 98.58                | 26.9                  |
|    | SiO <sub>2</sub>        | 18.1          | 0.42                 |                       |
|    | CaCO <sub>3</sub>       | 2.5           | 0.76                 |                       |
|    | Unidentified metaloxide | 0.1           | 0.24                 | no other assays made. |
|    |                         | 100.0         | 100.0                |                       |

The reasons for this change in behaviour are believed to include the following:

(a) The fluidity of the oleic acid collector agent complex at low temperatures makes possible the use of smaller quantities, giving high selectivity of reaction with the fluorite particles and assuring the avoidance of lumps of aggregated reagent in the pulp.

(b) The freely breaking and running froth can be manipulated so that mechanically entrained particles fall back into the pulp leaving very little beside pure fluorite to be removed as frothed mineral, because the small quantity of collector agent complex is still fluid, and the heavy edge-adhesion effects and obdurate flocculation frequently encountered in this work are prevented by the modification of the reagent.

(c) The improved dispersion of the collector agent complex during the pre-floatative conditioning stages of treatment aid the sought mineral in acquiring a monomolecular film of collector, and this increases the technical control of the activating and depressing treatment, and renders conditioning independent of the need for raised temperatures.

The process of the present invention offers the advantages, compared to previously known processes, that less oleic acid need be used, better grades of concentrate are produced, less heat need be applied to the pulp circuits, tailings losses are reduced, and technical control of the operation can more readily be effected.

Minerals which have been floated in tests made with the new collector agent complexes include the following:

Lead, in the form of cerussite (PbCO<sub>3</sub>),  
Lead-vanadium, in the form of descloizite and vanadinite,  
Zinc, in the form of smithsonite (ZnCO<sub>3</sub>),  
Tin, in the form of cassiterite (SnO<sub>2</sub>),  
Copper, in the form of malachite (CuCO<sub>3</sub>.Cu(OH)<sub>2</sub>).

These minerals were chosen as being minerals which are commonly met in the field and which present difficulties with standard flotation processes.

The tests were made in a Hallimond cell and pure minerals were treated at a pH approximately 7, using a concentration of the reagent P. F. 12 equivalent to 100 milligrams/litre. In each case the mineral floated and, as far as visual observation can show, flotation was better than with any known standard reagent used for these ores.

Whilst many of the metal sulphide minerals can be floated successfully with the aid of xanthate reagents, sphalerite (ZnS) cannot be floated efficiently by means of xanthate reagents. Tests which we have made with sphalerite in the Hallimond flotation cell show, however, that it can be floated excellently with the agent P. F. 12.

Tests made with coal in a standard Fagergren cell show that coal may be floated excellently with the agent P. F. 12.

Gypsum was also tested with success as follows:

1,000 gms. of gypsum ore ground to pass through a 60-mesh screen (I. M. M.) were floated in a laboratory flotation machine using 2.0 lb./ton of P. F. 12 and gave the following result:

Concentrate ..... percent 98.8  
Gypsum ..... gms. 640

The following examples illustrate how the separation of minerals by froth flotation may be carried out by the process of the invention:

*Example 7*

The ore treated was a Stanhopeburn fluorspar giving the following head assay:

|                   | Per cent |
|-------------------|----------|
| CaF <sub>2</sub>  | 71.3     |
| Pbs               | 3.9      |
| CaCO <sub>3</sub> | 2.4      |
| SiO <sub>2</sub>  | 20.5     |
| Fe oxides         | 1.8      |
| Unidentified      | 0.1      |
|                   | 100.0    |

The ore was ground through a 60-mesh screen (I. M. M.). Galena was first floated off with a reagent combination consisting of potassium ethyl xanthate 0.2 lbs./ton of ore; cresylic acid 0.05 lb./ton; pH 7.5-8.0 adjusted with soda-ash. Five minutes conditioning followed by three minutes frothing removed about 99% of the galena, as a rough concentrate needing reclean.

The ore was then conditioned for five minutes with sodium silicate (1 lb./ton) and twice deslimed.

Separate lots of ore were then conditioned for five minutes with 0.75 lb./ton quebracho and 0.25 lb./ton potassium dichromate, and treated with different flotation reagents at temperatures shown in the table below and floated. One stage of scavenge and three of cleaning were applied to a rougher concentrate, and the following results were obtained:

| Test No.                        | 1          | 3          | 11      | 12      | 14        |
|---------------------------------|------------|------------|---------|---------|-----------|
| Collector agent                 | Oleic acid | Oleic acid | P. F. 6 | P. F. 8 | P. F. 10. |
| Temp., ° C.                     | 30         | 21         | 4.0     | 5.0     | 4.0.      |
| Conc. Assay (CaF <sub>2</sub> ) | 98.6       | 98.2       | 98.8    | 98.5    | 98.9      |
| Tail Assay (CaF <sub>2</sub> )  | 13.2       | 18.1       | 8.7     | 17.4    | 15.6      |
| Oleic acid (lbs./ton of ore)    | 6.0        | 3.0        | 2.4     | 2.2     | 2.8       |

At temperatures below 20° C., it was not economically possible to produce 97.5% concentrate using plain oleic acid as collector.

Tests Nos. 11, 12 and 14, which were carried out by the process of the invention show how the separation may be carried out at lower temperatures than when oleic acid alone forms the reagent as in Tests Nos. 1 and 3.

*Example 8*

A French ore containing:

|                                | Per cent |
|--------------------------------|----------|
| CaF <sub>2</sub>               | 57.4     |
| CaCO <sub>3</sub>              | 3.0      |
| SiO <sub>2</sub>               | 36.4     |
| Fe <sub>2</sub> O <sub>3</sub> | 2.8      |
| Unidentified                   | 0.4      |
|                                | 100.0    |

was ground and conditioned as described in Example 7 and then floated with the aid of the reagent P. F. 12 under the conditions set out above. The concentrate was recleaned twice only, and the following results were obtained:

|                                 |          |
|---------------------------------|----------|
| Test No                         | 15       |
| Collector agent                 | P. F. 10 |
| Temp., ° C                      | 10       |
| Conc. assay (CaF <sub>2</sub> ) | 98.4     |
| Tail assay (CaF <sub>2</sub> )  | 5.6      |
| Oleic acid (lbs./ton of ore)    | 2.8      |

*Example 9.—Cassiterite SnO<sub>2</sub>*

*Material treated.*—A partially concentrated Cornish cassiterite with the following (incomplete) analysis:

|                                | Per cent |
|--------------------------------|----------|
| SiO <sub>2</sub>               | 32       |
| Fe <sub>2</sub> O <sub>3</sub> | 51       |
| SnO <sub>2</sub>               | 16.6     |

Quebracho and sodium silicate were used as modifiers and the material was floated in a Fagergren 500-gms. laboratory flotation machine with stage additions totalling 3.0 lbs./ton of P. F. 12.

Results:

| Product               | Weight, percent | Assay percent SnO <sub>2</sub> | Distribution of SnO <sub>2</sub> , percent |
|-----------------------|-----------------|--------------------------------|--------------------------------------------|
| Rougher Concentrate   | 7.7             | 61.0                           | 28.4                                       |
| Scavenger Concentrate | 25.8            | 44.3                           | 68.8                                       |
| Tailing               | 66.5            | 0.7                            | 2.8                                        |
| Head                  | 100.0           | 16.6                           | 100.0                                      |

*Example 10.—Apatite 3 Ca<sub>3</sub>(PO<sub>4</sub>)<sub>2</sub>CaF<sub>2</sub>*

*Material treated.*—An iron-contaminated apatite sand from Uganda containing silica, zircon, magnetite, pyrochlore and barytes.

The ore was conditioned for ten minutes with 1.0 lb./ton H<sub>3</sub>PO<sub>4</sub> and 2.0 lbs./ton Na<sub>2</sub>SiO<sub>3</sub> as modifiers and 3.5 lbs./ton of P. F. 12 as collector. The flotation time was three minutes and no cleaning was carried out.

Results:

| Product     | Weight, percent | Percent Apatite in product | Distribution of Apatite |
|-------------|-----------------|----------------------------|-------------------------|
| Concentrate | 89.3            | 97.82                      | 93.7                    |
| Tailings    | 10.7            | 55.62                      | 6.3                     |
| Heads       | 100.0           | 93.26                      | 100.0                   |

*Example 11.—Magnetite from ferrosilicon*

*Material treated.*—Ferrosilicon medium used in the

heavy media separation of Swedish iron ore and contaminated with magnetite.

The material was conditioned for ten minutes with 2 lbs./ton of sodium phosphate and 2 lbs./ton of sodium silicate as modifiers and 3½ lbs./ton of P. F. 12 as collector. The rougher concentrate was cleaned once with ½ lb./ton of P. F. 12 and 1 lb./ton of Na<sub>2</sub>SiO<sub>3</sub>.

Results:

| Product             | Weight, percent | Assays, percent |                                | Distribution, percent |                                |
|---------------------|-----------------|-----------------|--------------------------------|-----------------------|--------------------------------|
|                     |                 | Fe-Si           | Fe <sub>3</sub> O <sub>4</sub> | Fe-Si                 | Fe <sub>3</sub> O <sub>4</sub> |
| Cleaner concentrate | 13.8            | 16.8            | 82.3                           | 2.8                   | 63.0                           |
| Cleaner tailings    | 0.7             | 45.2            | 34.8                           | 0.4                   | 2.0                            |
| Rougher tailings    | 85.5            | 92.6            | 7.4                            | 96.8                  | 35.0                           |
| Head                | 100.0           | 81.6            | 18.3                           | 100.0                 | 100.0                          |

What we claim is:

1. A process for the production of a collector agent complex for use in the separation of minerals by froth flotation, which comprises making an aqueous dispersion of one part by weight of a member of the group consisting of the free acids and the sodium salts of a mixture of petroleum sulphonic acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; mixing said aqueous dispersion with an aqueous solution of one-third to 8 parts by weight of sodium silicate; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

2. A process for the production of a collector agent complex for use in the separation of minerals by froth flotation, which comprises making an aqueous dispersion of one part by weight of a member of the group consisting of the free acids and the sodium salts of a mixture of petroleum sulphonic acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; mixing said aqueous dispersion with an aqueous solution of one-half to 5 parts by weight of sodium silicate; adding water to give an aqueous suspension containing a total quantity of water varying within the range of 15 to 50 parts by weight in direct proportion to the quantity of oleic acid subsequently added; bringing 10 to 50 parts by weight of liquid oleic acid gradually into reaction with said last-mentioned aqueous dispersion by agitation of the mixture at an initial temperature of at least 50° C.; and continuing agitation until the product is homogeneous on standing.

3. A new, partly water-soluble, collector agent complex, wholly dispersible in water to form a stable emulsion, comprising a complex formed from oleic acid by making an aqueous dispersion of one part by weight of a member of the group consisting of the free acids and the sodium salts of a mixture of petroleum sulphonic acids obtained by sulphonation of a high-boiling petroleum fraction, the said mixture being characterized by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; mixing said aqueous dispersion with an aqueous solution of one-third to 8 parts by weight of sodium silicate; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

4. A method of separating minerals one from another which comprises subjecting a mixture of said minerals to froth flotation in the presence of an oleic acid collector agent complex formed by making an aqueous dispersion of one part by weight of a member of the group consisting of the free acids and the sodium salts of a mixture of petroleum sulphonic acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; mixing said aqueous dispersion with an aque-

ous solution of one-third to 8 parts by weight of sodium silicate; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

5. A method of separating fluorite from an ore containing fluorspar, which comprises subjecting said ore to froth flotation in the presence of an oleic acid collector agent complex formed by making an aqueous dispersion of one part by weight of a member of the group consisting of the free acids and the sodium salts of a mixture of petroleum sulphonic acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; mixing said aqueous dispersion with an aqueous solution of one-third to 8 parts by weight of sodium silicate; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

6. A process for the production of a collector agent complex for use in the separation of minerals by froth flotation, which comprises making an aqueous dispersion of one part by weight of the sodium salts of a mixture of petroleum sulphonic acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

7. A process for the production of a collector agent complex for use in the separation of minerals by froth flotation, which comprises making an aqueous dispersion of one part by weight of the sodium salts of a mixture of petroleum sulphonic acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; adding water to give an aqueous suspension containing a total quantity of water varying within the range of 15 to 50 parts by weight in direct proportion to the quantity of oleic acid subsequently added; bringing 10 to 50 parts by weight of liquid oleic acid gradually into reaction with said last-mentioned aqueous dispersion by agitation of the mixture at an initial temperature of at least 50° C.; and continuing agitation until the product is homogeneous on standing.

8. A new, partly water-soluble, collector agent complex, wholly dispersible in water to form a stable emulsion, comprising a complex formed from oleic acid by making an aqueous dispersion of one part by weight of the sodium salts of a mixture of petroleum sulphonic acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium

salts; heating said aqueous dispersion to boiling; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

9. A method of separating minerals one from another which comprises subjecting a mixture of said minerals to froth flotation in the presence of an oleic acid collector agent complex formed by making an aqueous dispersion of one part by weight of the sodium salts of a mixture of petroleum sulphonated acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; adding water to give an aqueous suspension containing a total quantity of water carrying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

10. A method of separating fluorite from an ore con-

taining fluorspar, which comprises subjecting said ore to froth flotation in the presence of an oleic acid collector agent complex formed by making an aqueous dispersion of one part by weight of the sodium salts of a mixture of petroleum sulphonated acids obtained by sulphonation of a high-boiling petroleum fraction, the said mixture being characterised by the solubility of its sodium salts in water, mineral hydrocarbon oils, oleic acid, benzene and chloroform, by partial solubility of said sodium salts in hydrochloric acid and by formation of water-insoluble calcium and barium salts; heating said aqueous dispersion to boiling; adding water to give an aqueous suspension containing a total quantity of water varying within the range of 8 to 50 parts by weight in direct proportion to the quantity of oleic acid subsequently added; bringing 2 to 50 parts by weight of liquid oleic acid gradually into reaction with said last-mentioned aqueous dispersion by agitation of the mixture at an initial temperature of at least 50° C.; and continuing agitation until the product is homogeneous on standing.

References Cited in the file of this patent

UNITED STATES PATENTS

| Number    | Name         | Date          |
|-----------|--------------|---------------|
| 1,678,311 | Adams        | July 24, 1928 |
| 2,069,365 | Handy        | Feb. 2, 1937  |
| 2,163,701 | Ried         | June 27, 1939 |
| 2,164,063 | Handy        | June 27, 1939 |
| 2,202,601 | Ried         | May 28, 1940  |
| 2,259,420 | Hills        | Oct. 14, 1941 |
| 2,433,258 | Booth et al. | Dec. 23, 1947 |